

U. S. ARMSTRONG.  
PROCESS OF COATING METAL ARTICLES.  
APPLICATION FILED FEB. 23, 1911.

1,012,048.

Patented Dec. 19, 1911.

2 SHEETS-SHEET 1.

FIG. 1.



FIG. 2.



FIG. 3.



FIG. 4.



FIG. 5.



FIG. 6.



witnesses:  
T. D. Humphries  
O. L. Thompson



Inventor:  
Alfred S. Armstrong  
By J. W. Cooke,  
attorney.

U. S. ARMSTRONG.  
PROCESS OF COATING METAL ARTICLES.  
APPLICATION FILED FEB. 23, 1911.

1,012,048.

Patented Dec. 19, 1911.

2 SHEETS-SHEET 2.



Witnesses:

J. B. Murphy,  
A. D. P. Miller.

Inventor:

Ulysses S. Armstrong  
By J. M. Cooksey  
Attorney.

# UNITED STATES PATENT OFFICE.

ULYSSES S. ARMSTRONG, OF NEW KENSINGTON, PENNSYLVANIA.

## PROCESS OF COATING METAL ARTICLES.

1,012,048.

Specification of Letters Patent. Patented Dec. 19, 1911.

Application filed February 23, 1911. Serial No. 610,367.

To all whom it may concern.

Be it known that I, ULYSSES S. ARMSTRONG, a resident of New Kensington, in the county of Westmoreland and State of Pennsylvania, have invented a new and useful Improvement in Processes of Coating Metal Articles; and I do hereby declare the following to be a full, clear, and exact description thereof.

10 My invention relates to the coating of metal articles, and has special reference to the coating of the interior and exterior surfaces of pipes or tubes.

The object of my invention is to provide 15 a cheap, simple and efficient process for the coating of metal articles, such as pipes or tubes, which will enable such articles to be coated on their inner and outer surfaces in a rapid and easy manner with a metallic 20 coating, such as lead and tin, or zinc, as well as enabling such a coating to be formed on such articles evenly and uniformly and without any waste of the material composing such coating.

25 To these ends my invention consists, generally stated, in the novel process employed in my improved coating of metal articles, as hereinafter more specifically set forth and described and particularly pointed out 30 in the claims.

To enable others skilled in the art to which my invention appertains to practice the process employed in my improved coating of metal articles, I will describe the 35 same more fully, referring to the accompanying drawing, in which—

Figure 1 is a top plan view of an apparatus employed in my improved process of coating metal articles. Fig. 2 is an end 40 view of the same. Fig. 3 is a cross section of the same on the line 3—3 Fig. 1. Fig. 4 is a longitudinal section of the same on the line 4—4, Fig. 1, looking in the direction of the arrow. Figs. 5 and 6 are views of the 45 swabbing devices employed. Fig. 7 shows another form of the device. Fig. 8 is a dia- grammatic plan view of the complete process employed.

Like symbols of reference herein indicate 50 like parts in each of the figures of the drawing.

As illustrated in the drawing, 1 represents the tank, which is provided with the usual heating furnace 1' under the same for 55 heating the materials within such tank for the coating of the articles to the desired de-

gree, and such tank is provided with the lower or base portion 2 and the upper portion 3 extending up from and at one side of said lower portion. Within the lower portion 2 of the tank 1 and extending longitudinally of the same and centrally thereof is a wall 4, which extends down from the top of the upper portion 3 and into said portion 2 for a suitable distance and divides such portion 2 into the compartments 5 and 6, as well as forming the inner side wall of the upper portion 3 located above the compartment 5. The wall 4 is provided with the projecting portions 7 and 8 at each end of the same, which extend from each side of said wall, and are adapted to form pockets 9 and 10 in said wall and on each side of the same for the purpose hereinafter described. Within the tank 1 are the two 75 shafts 11 and 12, one of which is placed on each side of such tank and preferably on an incline in parallel lines with each other. These shafts 11 and 12 are power driven in any suitable manner and are adapted to be 80 rotated or revolved in the same and in the proper direction, as shown by the arrows in Fig. 3. The shaft 11 is provided with a wheel 13 having radial arms 14 thereon at each end of the same, and the shaft 12 is 85 provided with a similar wheel 15 having similar arms 16 thereon at each end of the same. These wheels 13 and 15 are also arranged so that the ends of their respective arms 14 and 16 will travel within their respective pockets 9 and 10 in the wall 4 of the tank 1 in the movement of said wheels through said tank by the shafts 11 and 12, and are also arranged so that such arms on the end wheels 13 and 15 will overlap and 90 at the same time be away from each other by their being in the pockets 9 and 10 of the wall 4. When such arms 14 and 16 on the wheels 13 and 15 are in movement through the tank 1, the lower ends of the same will 95 pass along and be adjacent to the curved guides or bottoms 17 and 18 in the compartments 5 and 6 respectively of said tank, and such bottoms are connected together at their inner ends by the central raised portion 19 100 between the same.

The use and operation of my improved process of coating metal articles is as follows: The pipes or tubes *a* are cleaned in the usual manner by the pickling process in the tank A until the scale silicates and oxids are 110 loosened or removed from the surfaces of

the pipes, whereupon they are taken from said tank, placed on the truck A' and passed to the cleaning machine B, where the interiors of said pipes are further cleaned by running a revolving wire brush through the same and blowing air or steam through the pipe and brush, or by a sand blast, such as shown and described in my application filed May 5, 1911, Serial No. 625,373. After this cleaning operation has been completed the pipes are placed on the truck B' and passed forward to be repickled in a tank C containing a weakened solution of sulfuric or hydrofluoric acid, after which the pipes are then removed from the repickle and placed in a tank D of running water to prevent oxidation. The pipes are then taken from the tank of running water and while wet are each passed through a scrubbing machine E, which brushes the outside surface of the pipe, and such pipes are kept wet with cold water while passing through such machine. They are then passed down the inclined table F having rolls F' upon the same and pipes F<sup>2</sup> to spray the same with cold water, and are deposited in a storage tank G while wet, and such tank contains water and is located beside the coating machine 1, so that the pipe passes thus from the repickling tank through the running water tank and through the scrubbing machine to the storage tank while in a wet condition. The pipe is then taken from the storage tank and immediately dropped into the flux of the tank, as hereinafter described, while still in a wet condition, or the pipe may be fed automatically direct from the scrubbing machine to the coating machine by passing through water to prevent it from becoming dry and thus oxidize.

The compartments 5 and 6 of the portion 2 in the tank 1 are filled with the coating compound such as lead and tin, or zinc, which forms the coating bath b, and reaches the level of the wall 4, or slightly above the same, while the flux bath c of the usual material or compound for preparing the pipes or tubes a for the coating compound in the bath b is placed in the upper portion 3 of the tank and rests upon that part of the material of the coating bath b that is within the compartment 5 of said tank. The tank 1 being thus ready for the coating operation, the pipes a as so cleaned and wet from their immersion in cold water are each placed between two of the alined arms 14 on the wheels 13, as said wheels are revolved by the shaft 11, and such pipes are thus passed down through the flux bath c in the portion 3 of the said tank, and then they are passed by said wheels into the coating bath b in the compartment 5 of the lower portion 2 of said tank. When each of the pipes a carried by the arms 14 on the wheels 13

reach the raised portion 19 on the guides or bottoms 17 and 18 of the tank 1 they pass over said raised portion and are each caught by and between two of the alined arms 16 on the wheels 15, which wheels are being revolved in the same direction as the wheels 13, so that such arms will act to carry said pipes through the coating bath b in the compartment 6 of the lower portion 2 of said tank until they reach the upper part of said compartment and then each of said pipes are ejected from said compartment and out of said tank on the supporting table 20 at the side of said tank. As each one of the pipes a are thus passed through the flux bath c and coating bath b and are ejected from the tank 1, any surplus material from said bath b is drained from said pipes back into said bath and between the point where the pipe leaves the coating bath and the point where it assumes a horizontal position just before taking its place on the table 20, by reason of one end of such pipes being slightly elevated on account of the wheels 13 and 15 at one end of the tank 1 being so elevated and the coating compound entering said pipes in their passing from the bath c into the bath b being heavier than the flux will hold said flux at its level, so that it is kept in the flux bath c and does not thereby mix with said coating. When the pipes a are thrown out of the tank 1 after being so coated in the bath b and onto the asbestos coated table 20, each of the same can then be caught by any suitable means or mechanism and passed on to a suitable swabbing device 21, which is composed of a resilient collar or piston 22 of asbestos or other suitable material supported on a rod 23 and engaging with the interior of such pipe, while a die 24 on a base 25 and having a movable cover 26 over the same and provided with similar material 27 is adapted to engage with the exterior of such pipe to recover any further surplusage of the coating material upon such surfaces of said pipe, and to further coat any places on said pipe which may not have taken the molten coating while passing through said tank.

It will be obvious that the pipes are not allowed to become dry after being immersed in the cold water to wet the same and before they are placed in the usual muriatic acid and zinc solution, known as the flux, in order to avoid oxidation on such pipes taking place either in the air or in such flux before reaching the molten metal for coating the same.

It will be evident that the swabbing operation on both the interior and exterior surfaces of the pipes can be performed at one time as described, or at separate times, and by a continuous operation, as desired, while other articles than pipes

can be coated such as rods and bars, and other means, such as the sprocket and chain devices can be used in conveying the articles through the tank by a rotary movement instead of the rotating wheels, as shown in Fig. 7, by sprocket-wheels 13' and 15', chain 14' and arms 16' on said chain.

Various other modifications and changes in the process employed in my improved 10 coating of metal articles may be resorted to, without departing from the spirit of the invention, or sacrificing any of its advantages.

It will thus be seen that in my improved 15 coating of metal articles, such as pipes, the pipes in striking the coating compound in the first compartment at the bottom of the tank will drive the flux previously placed on such pipes ahead of the coating compound, which will permit such flux to remain above 20 said compound in its bath, and then such pipes are passed under the partition or wall into the second compartment and are raised out of the molten mixture or coating compound for the swabbing operation, all by 25 mechanical means, thereby enabling the rapid handling and coating of such pipes. With one end of the pipes being slightly elevated in passing through the tank, so as to incline such pipes, the material or ingredients composing the flux bath and coating bath to which such pipes are subjected will 30 always remain, or go back into their respective baths in the tank and thereby prevent any waste of such material, as well 35 as some of the material of the coating bath removed by the swabbing process can be saved into suitable pots or in any suitable devices, so that such pipe will receive a uniform and thin coating at the least possible expense. The apparatus shown being 40 automatic in its operation will not require any attention or handling of the pipes and will perform its work in a clean and workmanlike manner.

45 What I claim as my invention and desire to secure by Letters Patent is—

1. The process of coating metal articles comprising the steps of cleaning the article, then immersing the article in cold water, then 50 continuously passing the article while wet through a bath of flux and through a bath of metallic coating material, and then immediately removing the still soft surplus coating material from the surfaces of said 55 article.

2. The process of coating metal articles comprising the steps of cleaning the article, then immersing the article in cold water, then continuously passing the article while 60 wet through a bath of flux and through a bath of metallic coating material, and then immediately removing the still soft surplus coating material from the surfaces of said article by a swabbing operation.

65 3. The process of coating metal articles

comprising the steps of cleaning the article, then immersing the article in cold water, then continuously passing the article while wet through a bath of flux and through a bath of metallic coating material, and then 70 immediately removing the still soft surplus coating material from the surfaces of said article by a resilient swabbing operation.

4. The process of coating metal articles comprising the steps of cleaning the article, then immersing the article in cold water, then continuously passing the article while wet through a bath of flux and through a bath of metallic coating material on an incline, and then 75 immediately removing the still soft surplus coating material from the surfaces of said article.

5. The process of coating metal articles comprising the steps of cleaning the article, then immersing the article in cold water, then continuously passing the article while wet through a bath of flux and through a bath of metallic coating material on an incline, and then 85 immediately removing the still soft surplus coating material from the surfaces of said article.

6. The process of coating metal articles comprising the steps of cleaning the article, then immersing the article in cold water, then continuously passing the article while wet through a bath of flux and through a bath of metallic coating material on an incline, and then 95 removing the surplus coating material from the surfaces of said article by a resilient swabbing operation.

7. The process of coating metal articles comprising the steps of cleaning the article, then immersing the article in cold water, then continuously passing the article by a 105 rotary movement while wet through a bath of flux and through a bath of metallic coating material, and then immediately removing the still soft surplus coating material from the surfaces of said article.

8. The process of coating metal articles comprising the steps of cleaning the article, then immersing the article in cold water, then continuously passing the article by a rotary movement while wet through a bath 115 of flux and through a bath of metallic coating material, and then immediately removing the still soft surplus coating material from the surfaces of said article by a swabbing operation.

9. The process of coating metal articles comprising the steps of cleaning the article, then immersing the article in cold water, then continuously passing the article by a rotary movement while wet through a bath 125 of flux and through a bath of metallic coating material, and then removing the surplus coating material from the surfaces of said article by a resilient swabbing operation.

10. The process of coating metal articles 130



then continuously passing the pipe by a rotary movement while wet through a bath of flux and through a bath of metallic coating material on an incline, and then immediately removing the still soft surplus coating material from the exterior and interior surfaces of said pipe by a resilient swabbing operation.

24. The process of coating metal pipes comprising the steps of cleaning the article, then immersing the article in cold water, then continuously passing the pipe by a rotary movement while wet through a bath of

flux and through a bath of metallic coating material on an incline, and then immediately removing the still soft surplus coating material from the exterior and interior surfaces of said pipe by a resilient swabbing operation. 15

In testimony whereof, I, the said ULYSSES S. ARMSTRONG, have hereunto set my hand. 20

ULYSSES S. ARMSTRONG.

Witnesses:

T. B. HUMPHRIES,  
O. L. THOMPSON.